

Dec. 16, 1952

C. M. VAN BATTUM

2,622,112

PRODUCTION OF LUBRICATING OIL

Filed Oct. 9, 1950



Inventor: Carel M. Van Battum

By: Willard L. Caldwell  
His Attorney

## UNITED STATES PATENT OFFICE

2,622,112

## PRODUCTION OF LUBRICATING OIL

Carel M. Van Battum, Amsterdam, Netherlands,  
assignor to Shell Development Company, San  
Francisco, Calif., a corporation of Delaware

Application October 9, 1950, Serial No. 189,291  
In the Netherlands October 13, 1949

7 Claims. (Cl. 260—671)

1

This invention relates to the production of hydrocarbons useful as lubricating oils by the alkylation of aromatic hydrocarbons with olefins. It deals with an improved method of alkylation utilizing mixtures of aromatic hydrocarbons and olefinic mixtures to more efficiently produce high yields of lubricating oils having a combination of desirable properties.

It has been proposed (see, for example, British Patent 316,274) to produce viscous oils from aromatic hydrocarbon mixtures obtained by extracting mineral oil with liquid sulfur dioxide by reacting the extract with lower olefins such as ethylene and propylene in the presence of a Friedel-Crafts catalyst. It has also been suggested in British Patent 557,177 to prepare a pour point depressant for waxy lubricating oils by reacting an aromatic compound, preferably a polynuclear aromatic compound, such as naphthalene, with an olefin or a mixture of olefins with 5 to 9 carbon atoms, in the presence of a Friedel-Crafts catalyst, and by distilling off from the reaction product the components which boil below approximately 315° C.

Such methods of operation are not suitable for efficient production of lubricating oil when starting with mixtures of aromatic hydrocarbons of the kerosene boiling range and mixtures of 8 to 18 carbon atoms per molecule such as are obtained by cracking higher paraffin hydrocarbons. It has been found that with these readily available starting materials the yield of lubricating oil of satisfactory properties is prohibitively low. Thus, in experiments carried out by alkylating aromatic extracts prepared from kerosene and having a boiling range of from 140° C.—160° C. to 260° C.—280° C., in the presence of an aluminum chloride alkylation catalyst, with a mixture of olefins of 8 to 18 carbon atoms from the vapor phase cracking of paraffin wax, it was found that the products obtained after distilling off the unconverted components have the viscosity of a spindle oil but do not meet other specifications, particularly the flash point requirements, and are therefore not suitable for practical purposes. The Manufacturing Pool Specifications published in Great Britain, for instance, require a flash point (determined according to the Pensky-Martens closed cup method) of at least 201° C. for a lubricating oil with an Engler

2

viscosity of  $E_{50}=3$ , and a flash point of at least 204° C. for a lubricating oil with a viscosity of  $E_{50}=12$ . However, an alkylation product with a viscosity of  $E_{50}=5.1$ , prepared in the manner described above, was found to have a flash point of only 93° C. Even after distilling off the more volatile fractions from this alkylation product until the residue had a viscosity of  $E_{50}=14.2$ , the flash point of the residue so obtained was still found to be too low, viz. about 184° C. To obtain a lubricating oil with a sufficiently high flash point it would be necessary to remove such a large quantity of the more volatile components from the alkylation product that the yield of lubricating oil giving satisfaction in practice would be prohibitively low. Moreover, only high viscosity lubricating oils would be obtained in this way.

It is an object of the present invention to provide a method whereby high yields of lubricating oils having a satisfactory combination of properties, particularly desirable viscosity, viscosity index, flash point, pour point, stability and lubricating properties, can be obtained from mixtures of aromatic hydrocarbons of the kerosene boiling range and olefinic fractions having 8 to 18 carbon atoms per molecule. Other objects and advantages of the invention will be apparent from the following disclosure in which the use of aromatic extracts of kerosene will be emphasized as a particularly advantageous source of the aromatic hydrocarbon mixtures used as starting material, although it will be understood that analogous mixtures of aromatic hydrocarbons obtained in other ways can be similarly employed in the new process.

According to the present invention lubricating oil with a desirable combination of properties, particularly a high viscosity index and a satisfactory combination of viscosity and high flash point, is prepared from mixtures of aromatic hydrocarbons boiling in the range of between 140° C. and 280° C. such, for example, as those obtained by selective extraction of kerosene with solvents having a preferential solubility for aromatic hydrocarbons in the presence of paraffins, on the one hand, and mixtures of predominantly straight chain mono-olefins of 8 to 18 carbon atoms per molecule, on the other hand, by divid-

ing both the aromatic mixture and the olefinic mixture each separately as by distillation, for instance, into a lower boiling fraction and a higher boiling fraction, alkylating the lower boiling part of the aromatic extract with the higher boiling part of the mixture of olefins, alkylating the higher boiling part of the aromatic extract with the lower boiling part of the mixture of olefins, and mixing the alkylation products thus obtained. By mixing the two alkylation products in different proportions, this process makes it moreover possible to prepare lubricating oils of divergent viscosities, varying from about  $E_{50}=6$  to about  $E_{50}=18$ , having high viscosity indexes in combination with other desirable properties. These steps of the invention are shown in the flow sheet of the new process appearing in the accompanying drawing where only major operations are illustrated, and it will be understood that the schematic representations of the various steps are not intended to preclude ancillary or other operations.

The alkylation of the lower boiling fraction of the aromatic extract with the higher boiling fraction of the olefins is preferably carried out with a high molar ratio of aromatics to olefins. At least 2 mols, and preferably 2.5 to 3 mols, of aromatic compounds per mol of olefins should be present. Considerably larger quantities of the aromatic extract per mol of olefins can be applied, for example, 10 mols of aromatic compounds or more per mol of olefins. The preferred molecular ratio of 2.5:1 to 3:1 corresponds approximately to a weight ratio of aromatics to olefins of 1.6:1 to 2:1. The alkylation of the lower boiling fraction of the aromatic extract with the higher boiling fraction of the olefins produces a thin lubricating oil with a viscosity index of 95 to 110 and a sufficiently high flash point (above 200° C.).

In alkylating the higher boiling fraction of the aromatic extract with the lower boiling fraction of the olefins, preferably at least 2 mols of the latter are applied per mol of aromatic compounds. Usually 2 to 3, and most preferably about 2.5 mols of olefins are employed per mol of aromatic compounds. The molecular ratio of 2.5:1 corresponds approximately to a weight ratio of olefins to aromatic compounds of 3:1. The alkylation of the higher boiling fraction of the aromatic extract with the lower boiling fraction of the olefins produces a thick lubricating oil with a viscosity index of 95 to 105 and a sufficiently high flash point. If desired, the viscosity of this alkylation product can be further increased by distilling off the lighter components.

The point of division into higher boiling and lower boiling fractions of both the mixture of olefins and the aromatic extract can be varied considerably depending upon the particular type of lubricating oil which is desired. Thus, in the case of the olefin mixture, the splitting may be effected at any of the olefins with 11 to 17 carbon atoms. For the aromatic extract, the splitting into the lower and the higher boiling fractions can be carried out at any boiling point between 200° C. and 245° C. at atmospheric pressure. The splitting of the aromatic extract and of the starting mixture of olefins is advantageously carried out by distillation to these desired splitting points.

The aromatic extracts can be prepared by extracting the aromatic compounds from kerosene with a selective solvent. Liquid sulfur dioxide is particularly suitable as a selective solvent. How-

ever, other selective solvents for aromatic hydrocarbons in the presence of paraffins, such as furfural, nitrobenzene or antimony trichloride, can also be applied successfully. After extraction, the extract is separated from the residue and the selective solvent is removed from the extract. By distilling the extract thus obtained a fraction with an initial boiling point of 140° C.-160° C. and a final boiling point of 260° C.-280° C. can be isolated as the starting material for the new process. However, if desired, the extraction with a selective solvent can be replaced by other separation methods to concentrate the aromatic compounds from kerosene, for example, a percolation over silica gel of a kerosene diluted with a light hydrocarbon oil, such as pentane, whereafter the aromatic compounds adsorbed thereon are dissolved in a volatile solvent, such as pentane, which is finally distilled off. Still other methods of producing such starting mixtures of aromatic hydrocarbons boiling in the kerosene range can likewise be used.

It should be noted that not every kerosene which, on the ground of the ring analysis, has a high content of aromatic compounds forms a suitable initial material for the preparation of the alkylation products according to the invention. The aromatic compounds contained in the kerosene, or at least the greater part of them, must be alkylatable, i. e. must have a replaceable hydrogen atom attached to a nuclear carbon atom of the aromatic ring.

Suitable mixtures of olefins with 8 to 18 carbon atoms are, for example, those obtained by the cracking of heavy paraffin hydrocarbons, most preferably by cracking paraffin which is solid at room temperature in the gas phase and by distilling the C<sub>8</sub>-C<sub>18</sub> fraction out of the cracked product. It may be advisable to remove at least the majority of the very reactive components, such as di-olefins, from the cracked product before distilling off the C<sub>8</sub>-C<sub>18</sub> fraction by, for instance, bringing the cracked product into contact with a small proportion, for example 0.5% by weight, of aluminum chloride, preferably at a moderately elevated temperature, for example 60° C. to 90° C., which will cause these very reactive components to polymerize. After the aluminum chloride and any sludge formed have been removed, the C<sub>8</sub>-C<sub>18</sub> fraction is recovered from the product by distillation. Other methods of removing the undesired highly reactive components, if present, may also be used.

Strongly branched olefins, such as the polymer olefins obtained by the polymerization of lower olefins, are not suitable for the purpose of the invention in which, most preferably, C<sub>8</sub>-C<sub>18</sub> mixtures of predominantly straight chain alpha olefins are used as the starting material.

Of the two starting materials used, namely, aromatic extract and olefin mixture, the olefin mixture is usually the more expensive; consequently, it is generally desirable to adapt the consumption of the aromatic extract to that of the olefins so that the latter are consumed as completely as possible.

The two fractions of the aromatic extract are alkylated with the different fractions of the olefin mixture in the presence of an alkylation catalyst which may be the same or different in the two reactions. All the known Friedel-Crafts metal halide catalysts are effective for these alkylations, and aluminum chloride is particularly suitable. Aluminum halides can be used 75 as the anhydrous solid or in the form of com-

## 5

plexes or double salts or solutions in suitable solvents. Organic complexes of active metal halides with hydrocarbons are suitable and the complexes or sludges formed in the course of the reaction can, preferably after addition of fresh metal halide, be used as the catalyst. Other examples of suitable catalysts are, for instance, hydrogen fluoride, boron trifluoride, sulfuric acid, ferric chloride, and zinc chloride. The amount of catalyst which it will be desirable to use will vary depending upon the activity of the particular catalyst or catalyst mixture chosen. When using aluminum chloride, for example, as the catalyst, a quantity of about 0.5% to about 10% by weight thereof, based upon the total amount of reaction mixture present, is satisfactory. Most preferably, the proportion of aluminum chloride applied is 1% to 4% by weight for the alkylation of the lighter fraction of the aromatic extract with the heavier fraction of the olefins, and 4% to 6% by weight for the alkylation of the heavier fraction of the aromatic extract with the lighter fraction of the olefins.

The alkylation of the lighter fraction of the aromatic extract with the heavier fraction of the olefins can take place at temperatures varying from about 20° C. to about 100° C. and is preferably carried out at temperatures between about 20° C. and 70° C. The alkylation of the heavier fraction of the aromatic extract with the lighter fraction of the mixture of olefins can generally take place at temperatures from about -10° C. to about +100° C. and, generally, reaction temperatures of +10° C. to +50° C. are preferable.

The duration of the alkylation reactions is dependent on the temperature applied and the proportion and nature of the catalyst. If aluminum chloride is applied as catalyst and this catalyst is added gradually, the reaction time is usually from 3 to 8 hours. After completion of the reaction, the two alkylation products are worked up by first removing any bottom layer of catalyst sludge and higher molecular products. This can, for instance, be done by simply decanting or pumping off the top layer containing the alkylation product, or by separating the layers with the aid of a separatory funnel or by centrifugation.

The upper layer can then be treated with an alkaline substance, for instance, lime, to remove any acid components present. To improve the color of the alkylation product and to remove any chlorine content caused by the catalyst, the product can be treated with bleaching earth. The two treatments can be combined by heating the alkylation product with a mixture of bleaching earth and lime. A suitable heat treatment is, for example, the heating for 1/2 to 2 hours at a temperature between 150° C. and 240° C., preferably between 200° C. and 240° C. To prevent oxidation of the reaction product during this treatment, it can take place in an inert atmosphere, for example, an atmosphere of nitrogen. It is also possible to conduct nitrogen or another inert gas through the reaction product, which, at the same time, causes thorough stirring. After the treatment with lime and bleaching earth these substances are removed by filtration.

The filtrate can finally be subjected to a vacuum distillation to remove non-converted components of the initial materials. The recovered unreacted starting materials can be recycled for further reaction. The alkylates obtained as a result of the two alkylation reactions are finally mixed in the ratio which is necessary to obtain the lubricating oil of the desired viscosity.

## 6

In this way it is possible to prepare lubricating oils with any viscosity between  $E_{50}=6$  and  $E_{50}=18$ , a viscosity index of approximately 100, and a flash point above 200° C.

5 The following examples illustrate suitable methods of carrying out the new process when using a kerosene extract having a boiling range of 160° C. to 260° C. with a mixture of olefins of 8 to 18 carbon atoms, and show its advantages over direct alkylation of the extract with the olefin mixture.

10 The aromatic extract used was obtained from kerosene by extraction with liquid sulfur dioxide, and the mixture of olefins of 8 to 18 carbon atoms was produced by cracking a residual, oil-containing paraffin wax in the vapor phase, treating the cracked product for 3 hours at 80° C. with 0.5% by weight of aluminum chloride to remove the most reactive components, such as di-olefins, 15 and isolating the C<sub>8</sub>-C<sub>18</sub> fraction by vacuum distillation from the cracked product, after removing the catalyst and the sludge formed.

15 The kerosene extract was separated into two fractions by distillation to form a fraction with a boiling range of 160° C. to 210° C. and a fraction boiling 210° C. to 260° C. The mixture of olefins was divided into two fractions in each of four different distillations, which in each case split the mixture into a fraction with a chain length of 20 C<sub>8</sub>-C<sub>n</sub> and a fraction with a chain length of C<sub>n+1</sub>-C<sub>18</sub>, whereby n was 11, 13, 15, and 17 successively. In all the experiments the two olefin fractions were used in the same ratio as that in which they were present in the entire C<sub>8</sub>-C<sub>18</sub> 25 mixture, while two parts by weight of the lighter fraction of the kerosene extract were reacted with one part by weight of the C<sub>n+1</sub>-C<sub>18</sub> olefins and one part by weight of the heavier fraction of the kerosene extract was reacted with three 30 parts by weight of the C<sub>8</sub>-C<sub>n</sub> olefins.

35 Eight alkylations were carried out in pairs in which the lower boiling fraction of the aromatic extract was reacted with a higher boiling fraction of the olefin mixture and the corresponding lower 40 boiling fraction of the olefin mixture was reacted with the higher boiling fraction of the aromatic extract. Each alkylation was carried out in a stirred autoclave at 45° C. using 3.6% by weight of aluminum chloride based on the total weight 45 of the reaction mixture and a total reaction time of about 4 to 5 hours.

50 At the end of the reaction two layers had formed in the reaction mixture. The bottom layer, consisting of catalyst sludge, was removed. The upper layer was treated with 10 parts by weight of an aqueous sodium hydroxide solution of 20% concentration and washed with water after the aqueous alkali layer has been removed.

55 The oils obtained by alkylating the fraction of the kerosene extract having a boiling range of 160° C.-210° C. with the C<sub>n+1</sub>-C<sub>18</sub> olefins were distilled off to a viscosity of  $E_{50}=\text{approx. } 4$ , so as to remove non-converted components of the initial mixture; the oils thus obtained had a flash point higher than 200° C. and a viscosity index between 60 95 and 110.

65 The products obtained by alkylating the fraction of the kerosene extract having a boiling range of 210° C.-260° C. with the C<sub>8</sub>-C<sub>n</sub> olefins were distilled off after the completion of the alkylation reaction to a viscosity of  $E_{50}=25$ , so as to remove lighter components (including non-converted components of the initial mixture). 70 The oils thus obtained had flash points of 75

230° C.-240° C. and a viscosity index between 95 and 105.

The parts by weight of olefins brought into reaction and the parts by weight of lubricating oil obtained therefrom as well as the flash points of the mixtures finally obtained were for the different values of  $n$  as follows:

| $n$ | Quantity of olefins                               | Quantity lub. oil obtained | Total quantity lub. oil after mixing | Visc. of the lub.   | Flash point oil mixture |
|-----|---------------------------------------------------|----------------------------|--------------------------------------|---------------------|-------------------------|
| 11  | { 32 parts C <sub>8</sub> -C <sub>11</sub> .....  | 30                         | Parts                                | E <sub>50</sub> =6  | 204                     |
|     | { 68 parts C <sub>12</sub> -C <sub>18</sub> ..... | 78                         | 108                                  |                     |                         |
| 13  | { 48 parts C <sub>8</sub> -C <sub>13</sub> .....  | 45                         | 105                                  | E <sub>50</sub> =8  | 208                     |
| 15  | { 52 parts C <sub>14</sub> -C <sub>18</sub> ..... | 60                         |                                      |                     |                         |
|     | { 69 parts C <sub>8</sub> -C <sub>15</sub> .....  | 66                         | 101                                  | E <sub>50</sub> =12 | 213                     |
| 17  | { 31 parts C <sub>16</sub> -C <sub>18</sub> ..... | 35                         |                                      |                     |                         |
|     | { 89 parts C <sub>8</sub> -C <sub>17</sub> .....  | 85                         | 99                                   | E <sub>50</sub> =18 | 223                     |
|     | { 10.4 parts C <sub>13</sub> .....                | 14                         |                                      |                     |                         |

In the third column of this table the quantities of lubricating oil obtained in each of the two alkylation reactions are indicated separately, while the fourth column shows the total quantity of lubricating oil obtained by mixing these quantities. The fifth column shows the viscosities expressed in degrees Engler at 50° C. of the products obtained after this mixing, while finally the sixth column shows the flash points of these mixtures. The viscosity index of each of these mixtures was approximately 100.

When the same starting aromatic extract of boiling range 160° C.-260° C. without fractionation was reacted with the same starting mixture of olefins of 8 to 18 carbon atoms, also unfractionated, in the proportions of 30 parts of extract to 70 parts of olefin mixture by weight, under the same conditions, the finished product recovered in the same way failed to meet the specifications for a satisfactory lubricating oil, particularly in respect to proper relationship of flash point and viscosity. In an effort to improve the product, it was distilled to remove a part, and the flash point and viscosity of the residue were again determined. The properties of the residue being still unsatisfactory, further distillations were carried out with the following results:

| Product                  | Yield, wt. percent of the original mixture of olefins | Flash-Point (Fensky-Martens closed cup) | Visc., 37° C., in c. s. | Visc., 99° C., in c. s. | E <sub>50</sub> |
|--------------------------|-------------------------------------------------------|-----------------------------------------|-------------------------|-------------------------|-----------------|
| Original final prod..... | 123.0                                                 | 93                                      | 64.95                   | 8.94                    | 5.13            |
| Residue I.....           | 111.2                                                 | 142                                     | 124.50                  | 13.30                   | 9.09            |
| Residue II.....          | 100.4                                                 | 184                                     | 206.96                  | 18.05                   | 14.23           |
| Residue III.....         | 90.8                                                  | 216                                     | 317.85                  | 23.73                   | 20.94           |
| Residue IV.....          | 79.9                                                  | 242                                     | 476.89                  | 30.77                   | 30.49           |
| Residue V.....           | 69.1                                                  | 263                                     | 694.8                   | 40.47                   | 43.0            |

A comparison of these results with those obtained by the process of the invention shows the advantages of the new method, especially in giving lubricating oil of a considerably higher flash point at a given viscosity. The new lubricating oils produced by splitting the aromatic extract and olefinic mixtures, alkylating in two steps the lighter fraction of the aromatic extract with the heavier fraction of the olefins and vice versa, and blending the alkylates, show other unexpected improvements. Thus, from engine tests it has been found that the new lubricating oil blends

produce less deposits in engines than do each of the components individually.

These tests were carried out with lubricating oils prepared as follows:

- 5 A fraction of an aromatic extract of kerosene boiling from 160° C. to 210° C. was alkylated with a C<sub>14</sub>-C<sub>18</sub> fraction of cracked wax olefins in the ratio of two parts by weight of the aromatic extract fraction to one part by weight of the olefin fraction. The alkylation product was distilled off to obtain a light component having a viscosity of E<sub>50</sub>=4. The higher boiling fraction of the aromatic extract, boiling range 210° C.-260° C., was alkylated with the C<sub>8</sub>-C<sub>13</sub> fraction of the olefins in the ratio of one part by weight of aromatic fraction to three parts by weight of the olefins, and the alkylation product distilled off to obtain a heavy component having a viscosity of E<sub>50</sub>=25.

10 Three engine tests were now carried out, using 20 as lubricating oil (1) the light component, (2) the heavy component, and (3) a mixture of the light and the heavy components. In the first 25 test, using only the light component as lubricating oil, the lighter components of the oil were first distilled off to obtain a residue having a viscosity of E<sub>50</sub>=14 to make the viscosity properties of the lubricating oil better comparable with those of the heavy component and the mixture of light and heavy components. The mixture of 30 light and heavy components was a mixture of 20 parts by weight of the light component with a viscosity of E<sub>50</sub>=4 and 80 parts by weight of the heavy component (E<sub>50</sub>=25), which mixture had a viscosity of E<sub>50</sub>=18.

35 The tests were carried out in a stationary single cylinder Deutz gasoline engine under full load (100 mm. bore, stroke 110 mm.). The engine was operated under the following conditions:

40 Cooling temperature (glycol as cooling liquid) ..... °C. 190  
Oil temperature ..... °C. 80  
Engine speed ..... R. P. M. 1200

45 The tests were of 40 hours' duration and the following results were obtained:

|                                    | Deposit | Thickened Light Component | Heavy Component | Mixture of Light and Heavy Components |
|------------------------------------|---------|---------------------------|-----------------|---------------------------------------|
| 50                                 |         |                           |                 |                                       |
| 1st piston-ring groove.....        | mg.     | 109                       | 48              | 24                                    |
| 2nd piston-ring groove.....        | mg.     | 12                        | 35              | 0                                     |
| Remaining piston-ring grooves..... | mg.     | 5                         | 20              | 0                                     |
| 55 Inside the piston.....          | mg.     | 222                       | 0               | 0                                     |

It will thus be seen that the new process of the invention offers many advantages over prior methods of synthesizing lubricating oils and that the process is capable of considerable variation, not only in regard to the starting materials which may be used but also in respect to the methods of operation which may be adopted. Thus, while pure or relatively pure mixtures of alkylatable aromatic hydrocarbons of the kerosene boiling range, such as are obtained by extraction of kerosene with suitable solvents, are particularly suitable for the process, it is also possible to use less pure mixtures of such aromatic hydrocarbons. For instance, instead of extracting the desired aromatic hydrocarbons from the kerosene before operation according to the invention, one can start with a substantially olefin-free kerosene boiling mixture rich in aromatics, distill it to separate lower and higher boiling

fractions with the split point between 200° C. and 245° C., separately alkylate these fractions with higher and lower boiling fractions of olefins as previously described, and separate from the alkylation products by distillation the non-aromatic components of the kerosene fractions which have not taken part in the alkylation before blending the alkylates to obtain the desired lubricating oil of high quality. The alkylations may be carried on continuously, intermittently or batchwise. The new products of the invention may be employed with any of the known lubricating oil additives such, for instance, as anti-oxidants, or with other lubricants or the like, although their advantageous combination of properties make them also useful without the addition of other components. Still other variations may be made in the process which is not limited by the examples given by way of illustration nor by any theory proposed in explanation of the improved results which are obtained.

I claim as my invention:

1. A method of producing aromatic hydrocarbons useful as lubricating oil from a mixture of aromatic hydrocarbons boiling in the kerosene range and a mixture of predominantly straight chain olefins having 8 to 18 carbon atoms per molecule, which comprises separating said aromatic mixture into two fractions, one of which boils higher than the other, separating said olefin mixture into a lower boiling fraction and a higher boiling fraction, alkylating said higher boiling fraction of the aromatic mixture with the lower boiling fraction of said olefin mixture, alkylating the lower boiling fraction of the aromatic mixture with said higher boiling fraction of the olefin mixture, and blending alkylation products of the two said alkylations.

2. A method of producing aromatic hydrocarbons useful as lubricating oil from a mixture of aromatic hydrocarbons having an initial boiling point within the range of from 140° C. to 160° C. and a final boiling point within the range of from 260° C. to 280° C. and a mixture of olefins of 8 to 18 carbon atoms per molecule obtained by cracking higher paraffin hydrocarbons, which comprises distilling said mixture of aromatic hydrocarbons to separate two fractions, the lower boiling of which has an upper boiling limit between 200° C. and 245° C. at atmospheric pressure and the higher boiling fraction of which is the remainder of said aromatic mixture, dividing said mixture of olefins into a  $C_8-C_n$  fraction and a  $C_{n+1}-C_{18}$  fraction, where  $n$  is a number from 11 to 17, alkylating said higher boiling fraction of the aromatic mixture with the  $C_8-C_n$  fraction of the olefin mixture, alkylating the lower boiling fraction of the aromatic mixture with the  $C_{n+1}-C_{18}$  fraction of olefins, and blending alkylation products therefrom to form a lubricating oil having a viscosity of  $E_{50}=6$  to  $E_{50}=18$ .

3. A method of producing aromatic hydrocarbons useful as lubricating oil from a mixture of aromatic hydrocarbons having an initial boiling point within the range of from 140° C. to 160° C. and a final boiling point within the range of from 260° C. to 280° C. and a mixture of predominantly straight chain olefins having 8 to 18 carbon atoms per molecule, which comprises separating said aromatic mixture into two fractions, the lower boiling of which boils in the range of 140° C. to 245° C. and has a final boiling point within the range of from 200° C. to 245° C. and the higher boiling of which boils in the range of

200° C. to 280° C. and has an initial boiling point within the range of from 200° C. to 245° C., dividing said mixture of olefins into a  $C_8-C_n$  fraction and a  $C_{n+1}-C_{18}$  fraction, where  $n$  is a number from 11 to 17, reacting a mixture of said lower boiling aromatic fraction and said  $C_{n+1}-C_{18}$  fraction of olefins containing at least two mols of aromatic hydrocarbons per mol of olefin under alkylation conditions in the presence of an alkylation catalyst, reacting said higher boiling fraction of the aromatic mixture with said  $C_8-C_n$  fraction of olefins in a ratio of at least two mols of olefin per mol of aromatic hydrocarbon present under alkylation conditions in the presence of an alkylation catalyst, and blending alkylation products therefrom to form a lubricating oil having a viscosity of  $E_{50}=6$  to  $E_{50}=18$ .

4. A method of producing aromatic hydrocarbons useful as lubricating oil from a mixture of aromatic hydrocarbons boiling in the kerosene range and a mixture of predominantly straight chain olefins having 8 to 18 carbon atoms per molecule, which comprises separating said aromatic mixture into two fractions, one of which boils higher than the other, separating said olefin mixture into a lower boiling fraction and a higher boiling fraction, alkylating said higher boiling fraction of the aromatic mixture by reaction with the lower boiling fraction of said olefins in the ratio of 2 to 3 mols of olefins per mol of aromatic hydrocarbon, at a temperature of -10° C. to 50° C. in the presence of 4% to 6% by weight of aluminum chloride based upon the weight of reaction mixture, alkylating the lower boiling fraction of said aromatic mixture with the higher boiling fraction of said olefins in the ratio of 2.5 to 3 mols of aromatic hydrocarbon per mol of olefin, at a temperature of 20° C. to 70° C. in the presence of 1% to 4% of aluminum chloride based on the weight of the reaction mixture, and blending alkylation products of the two reactions.

5. A process according to claim 4 wherein the mixture of aromatic hydrocarbons is a liquid sulfur dioxide extract of kerosene.

6. A method of producing aromatic hydrocarbons useful as lubricating oil from a mixture of aromatic hydrocarbons having an initial boiling point within the range of from 140° C. to 160° C. and a final boiling point within the range of from 260° C. to 280° C. and a mixture of olefins of 8 to 18 carbon atoms per molecule obtained by cracking higher paraffin hydrocarbons, which comprises distilling said mixture of aromatic hydrocarbons to separate two fractions, the lower boiling of which has an upper boiling limit between 200° C. and 245° C. at atmospheric pressure and the higher boiling fraction of which is the remainder of said aromatic mixture, dividing said mixture of olefins into a  $C_8-C_n$  fraction and a  $C_{n+1}-C_{18}$  fraction, where  $n$  is a number from 11 to 17, alkylating said higher boiling fraction of the aromatic mixture with the  $C_8-C_n$  fraction of olefins in the ratio of 2 to 3 mols of olefins per mol of aromatic hydrocarbon, at a temperature of -10° C. to 50° C. in the presence of 4% to 6% by weight of aluminum chloride based upon the weight of reaction mixture, alkylating the lower boiling fraction of said aromatic mixture with the  $C_{n+1}-C_{18}$  fraction of olefins in the ratio of 2.5 to 3 mols of aromatic hydrocarbons per mol of olefin at a temperature of 20° C. to 70° C. in the presence of 1% to 4% of aluminum chloride based on the weight of reaction mixture, and blending alkylation

11

products therefrom to form a lubricating oil having a viscosity of  $E_{50}=6$  to  $E_{50}=18$ .

7. A process according to claim 6 wherein the more reactive components of the cracking product are removed by selective polymerization with a small amount of aluminum chloride before carrying out said alkylations.

CAREL M. VAN BATTUM.

## REFERENCES CITED

The following references are of record in the file of this patent:

12

## UNITED STATES PATENTS

| Number    | Name             | Date          |
|-----------|------------------|---------------|
| 2,071,521 | Hartmann et al.  | Feb. 23, 1937 |
| 2,232,118 | Kyrides          | Feb. 18, 1941 |
| 2,360,446 | Reid             | Oct. 17, 1944 |
| 2,518,529 | De Casson et al. | Aug. 15, 1950 |

## OTHER REFERENCES

- 10 Hall, "Research on Synthetic Lubricants," Oil and Gas Jour. (Mar. 28, 1935), pp. 81, 82, 96 (3 pages).